

July 27, 1971

H. N. VAZIRANI

3,595,708

PROCESS FOR SURFACE TREATMENT OF IRON AND ITS ALLOYS

Filed Nov. 12, 1968

FIG. 1



FIG. 2



INVENTOR  
H.N. VAZIRANI  
BY  
*George S. Brody*  
ATTORNEY

## 1

3,595,708

### PROCESS FOR SURFACE TREATMENT OF IRON AND ITS ALLOYS

Hargovind N. Vazirani, Passaic Township, Morris County, N.J., assignors to Bell Telephone Laboratories, Incorporated, Murray Hill, N.J.

Filed Nov. 12, 1968, Ser. No. 774,930

Int. Cl. C23f 7/10

U.S. Cl. 148—6.15

8 Claims

#### ABSTRACT OF THE DISCLOSURE

Treating the surface of iron and its alloys with an aqueous solution containing bromide ions or iodide ions and phosphoric acid results in improved surface for adhesive joining and for coating with organic finishes. Effectiveness of the treatment on highly corrosion resistant steels is somewhat improved by the addition of minor amounts of sulfuric acid to the solution.

#### BACKGROUND OF THE INVENTION

##### (1) Field of the invention

This invention relates to the surface treatment of iron and its alloys by the use of an acid aqueous solution containing bromide ions or iodide ions, in order to improve joints subsequently formed with organic materials, and also relates to the joined product.

##### (2) Description of the prior art

Joining iron and its alloys to organic materials is desirable in many cases, as for example, in the adhesive joining and protective coating of steel structural parts. Corrosion products ordinarily present on the surface of the metal interfere with such joining and have in the past been removed both chemically, as for example, by hydrochloric acid treatment, and mechanically, as for example, by abrasive blasting.

Mechanical abrasion is generally undesirable because it is wasteful of the metal surface and produces a rough texture which gives rise to localized stresses in subsequently formed joints when placed under stress.

Chemical cleaning is less damaging to the surface of the metal. In addition, the corrosion products may be replaced by a chemically produced oxide layer which prevents further corrosion and provides a surface suitable for joining. This layer has been achieved, for example, by the use of an oxidizing agent such as hydrogen peroxide, as disclosed in U.S. Pat. 2,923,608. However, joints subsequently formed on such surfaces often degrade with time resulting in eventual joint failures. Depending on the temperature, stress and humidity levels, such failures may occur after only a few days.

#### SUMMARY OF THE INVENTION

This invention is essentially a joining technique in which the surfaces of iron and its alloys are treated with a solution containing bromide ions or iodide ions and phosphoric acid prior to joining. Such treatment results in removal of corrosion products and their replacement by a mechanically strong protective layer thus enabling joints to be formed which exhibit excellent initial strengths and which resist degradation with time.

The invention encompasses treating solutions containing minor addition of sulfuric acid, preferred for treatment of high corrosion-resistant steels.

Since the surface to be treated ordinarily contains contaminants such as dirt, grease and corrosion products, it is usually necessary to remove these prior to the surface treatment and to aid the practitioners, exemplary procedures are briefly described.

## 2

#### BRIEF DESCRIPTION OF THE DRAWING

FIG. 1 is a cross-sectional view of a two part laminate formed according to the inventive process; and

FIG. 2 is a cross-sectional view of a three part laminate formed according to the inventive process.

#### DETAILED DESCRIPTION

This process applied to iron and any of its alloys containing at least 50% iron, and has as its principal object the removal of dirt and corrosion products from the metal surface and replacement with a chemically produced layer. Since an object of the surface treatment is to remove oxide scale, any advantage to be gained by preliminary cleaning of the metal surface will ordinarily reside in the reduced rate of contamination of the treating solution, replacement of which may be both costly and time consuming.

Preliminary cleaning is by methods well known in the art. Thus, the following description of preliminary cleaning is intended to be exemplary and not limiting.

Preliminary cleaning is generally divided into degreasing and descaling. For example, degreasing is generally effective in removing only oils and grease and is ineffective in removing corrosion products such as naturally formed oxide scale. Descaling, which may be either mechanical or chemical, will, however, generally remove substantially all of the surface contamination. However, descaling chemically without first degreasing may result in rapid contamination of the solution.

Removal of oils and grease may be accomplished by the use of organic solvents such as alcohols, ketones and chlorinated solvents such as trichloroethylene and perchloroethylene, or by the use of well known alkaline cleaners.

Scaling is usually accomplished by the use of acid solutions or by mechanical abrasion. However, where joints of high initial strength and high resistance to degradation are desired, it is preferred to avoid mechanical abrasion, strong chemical etchants, or other descaling methods which would result in rough or pitted metal surfaces.

A more complete description of degreasing and descaling methods may be found in Protective Coatings for Metals, third edition, American Chemical Society, Monograph 163, by R. M. Burns and W. W. Bradley, pp. 27 to 54, in Reinhold (1967).

Once the preliminary removal of surface contamination has been effected, the clean metal surface should be either treated promptly to form the desired protective layer or stored under noncorrosive conditions until treatment in order to realize any advantage gained, since exposure of the clean surface to a nonprotective atmosphere will soon result in reformation of corrosion products.

Formation of the protective layer may be carried out by contacting the metal surface with a treating solution containing bromide or iodide ions in the range from 0.001% by weight to saturation although from 1 to 10% of iodide is preferred for optimum results. The ions may be introduced in combination with the Group I alkali metals; lithium, sodium, potassium, rubidium and cesium or the Group II alkaline earth metals; beryllium, magnesium, calcium, strontium and barium.

The phosphoric acid should generally be present in the treating solution in a concentration sufficient to etch the metal uniformly typically 30 to 70%, below which uneven etching or even pitting is likely to occur, and above which the rate of attack of the metal surface is impractically slow. A concentration of from 40 to 60% of  $H_3PO_4$  is preferred, based on these considerations.

The phosphoric acid solution containing iodide ions is intended primarily for use with the less corrosion-resistant steels, such as cold rolled steels and the high

strength steels. Highly corrosion-resistant or "stainless" steels, not only resist the action of the treating solution, but also generally require less critical surface treatment preparatory to joining. However, if it is desired to treat highly corrosion-resistant surfaces, a strongly etching acid, such as  $H_2SO_4$ , may be added to the treating solution in amounts up to about 5%, beyond which formation of a rough, pitted surface is likely.

The degree of attack of the surface will in general increase with increasing time of treatment or temperature of solution. Accordingly, at high temperatures, relatively short treatment times should be used. At 230° F., constituting an upper limit beyond which boiling or decomposition of the solution will occur, the time of treatment should generally not exceed two minutes, while at room temperature, treatment times of about ten minutes are tolerable. For optimum results, a preferred range is from three to five minutes at about 160° to 200° F.

The following examples compare adhesive joint strengths obtained by the inventive treatment and by various other treatments.

#### EXAMPLE 1

Four sets of standard lap joints were made from specimens of No. 1010 (about 0.1% carbon) cold rolled steel (having dimensions of about one inch in width and sixty-three mils in thickness) and an epoxy adhesive, claimed to give strong joints without surface treating. Treatment prior to joining was as follows: Set 1 was not treated. All of the specimens in sets 2, 3, and 4 were vapor degreased. Set 3 was then grit blasted with alumina powder. Set 4 was treated for five minutes in a solution containing 5% by weight of KI and 50% by volume conc.  $H_3PO_4$  at 180° F., and rinsed with deionized water. The results are shown in Table 1 as the initial joint strength in pounds per square inch and time to failure when a static load of 1500 pounds per square inch was applied in an ambient atmosphere of 95° F. at 90% relative humidity.

TABLE 1

|                                              | 1     | 2     | 3     | 4     |
|----------------------------------------------|-------|-------|-------|-------|
| Initial joint strength (p.s.i.)              | 2,900 | 2,910 | 4,260 | 4,470 |
| Days to failure, 1,500 p.s.i., static stress | 2     | 19    | 101   | 170   |

#### EXAMPLE 2

Two sets of standard lap joints were made from specimens of No. C-1095 (about 0.95% carbon) cold rolled steel as in Example 1. Treatment prior to joining was as follows: Set 1 was treated for five minutes in a solution containing 50% by volume of conc. HCl, and rinsed with deionized water. Set 2 was treated as was set 4 in Example 1. Results are shown in Table 2 in the same manner as shown in Table 1, except that time to failure was for a static load of 4000 p.s.i.

TABLE 2

|                                 | 1     | 2     |
|---------------------------------|-------|-------|
| Initial joint strength (p.s.i.) | 6,630 | 8,200 |
| Days to failure, 4,000 p.s.i.   | 12    | 48    |

The results of Tables 1 and 2 indicate that strong joints, desirable under static loading, are obtainable by use of the inventive treatment on cold rolled steel. The following example shows the beneficial effects of addition of  $H_2SO_4$  to the treating solution and of elevated treatment temperatures in the case of highly corrosion-resistant steel.

#### EXAMPLE 3

Three sets of standard lap joints were made from specimens of No. 302 steel (approximate composition; 0.15% carbon, 2% manganese, 1% silicon, 17 to 19% chromium, 8 to 10% nickel, remainder iron) as in Example 1. Treatment prior to joining was as follows: All specimens in each set were vapor degreased and alkaline cleaned.

Set 1 was then treated for five minutes in a solution containing 5% by weight KI and 50% by volume conc.  $H_3PO_4$  at 150° F. Set 2 was treated as was set 1, except that 10% of the conc.  $H_3PO_4$  was replaced by conc.  $H_2SO_4$ . Set 3 was treated as was set 2, except that the temperature of the solution was raised to 180° F. Results are shown in Table 3 in the same manner as shown in Table 2.

TABLE 3

|                                 | 1     | 2     | 3     |
|---------------------------------|-------|-------|-------|
| Initial joint strength (p.s.i.) | 6,400 | 6,730 | 7,450 |
| Days to failure, 4,000 p.s.i.   | 27    | 60    | 104   |

The invention has been described in terms of improving joints between iron and its alloys and organic materials. Such organic materials include adhesives, coatings and potting compounds. Examples of adhesive materials are epoxies and modified epoxy resins, nitrile rubber phenolics, polyvinyl butyral and polyvinyl formals. Examples of coating materials are alkyds and modified alkyds, acrylics, polyesters and urethanes. Potting compounds include polyurethanes, silicones and epoxies.

The following example indicates that coatings adhere well to metal surfaces treated according to the invention.

#### EXAMPLE 4

Three sets of No. 1010 cold rolled steel panels were treated as follows: All sets were vapor degreased. Set 2 was treated with a zinc phosphate solution and rinsed with a chromic acid solution, a commonly used treatment prior to coating. Set 3 was treated as was Set 4 in Example 1. All sets were then coated with about a  $\frac{1}{2}$  mil thick primer followed by about a 5 mil thick layer of a vinyl acrylic organosol. The coating was then fused at about 360° F. for twenty minutes, a standard coating technique. Results are shown in Table 4 in terms of visual appearance of coatings after salt spray according to ASTM test B117 and humidity cycling.

40

TABLE 4

|                              | 1                     | 2                 | 3                  |
|------------------------------|-----------------------|-------------------|--------------------|
| Salt spray (hrs.):           |                       |                   |                    |
| 96                           | Loose coating         | Loose coating     | No visible defects |
| 240                          | Blistering of coating | Slight blistering | Do.                |
| 500                          | Severe blistering     | Blistering        | Do.                |
| 1,700                        |                       |                   | Do.                |
| Humidity cycling (hrs.): 500 | Slight peeling        | Peeling           | Do.                |

Referring now to the drawing, there is shown a joined product prepared in accordance with the inventive process. Shown in the figure is an iron or iron alloy body 1, joined to an organic body 2.

In FIG. 2 is shown an iron or iron alloy body 10, joined to an organic body 11, and further joined to a metal body 12.

What is claimed is:

1. A method for preparing a surface containing at least 50% by weight iron for joining to an organic material, characterized in that said method comprises the step of contacting said surface with an aqueous solution consisting essentially of phosphoric acid in the amount of from 40 to 60% by weight and at least one member from the group consisting of bromide ions and iodide ions, said member being present in the amount of from 1 to 10% by weight and said member being introduced into the solution as a compound of an element selected from Groups I and II of the Periodic Table.

2. The method of claim 1 in which said solution additionally contains up to 5% by weight of sulfuric acid.

75

3. The method of claim 1 in which the step of contacting said surface with said solution is carried out at a temperature of up to 230° F. for up to two minutes.

4. The method of claim 3 in which said step of contacting said surface with said solution is carried out at a temperature of from 160 to 200° F. for from three to five minutes.

5. The method of claim 1 in which the step of contacting said surface with said solution is preceded by descaling.

6. The method of claim 1 in which the step of contacting said surface with said solution is followed by adhesive joining of an organic material to said surface.

7. The method of claim 6 in which the joining is for

the purpose of joining the surface to one or more other surfaces.

5 8. Product produced by the method of claim 1.

References Cited

UNITED STATES PATENTS

3,364,081 1/1968 Forsberg ----- 148—6.15  
2,514,149 7/1950 Amundsen ----- 148—6.15

10 RALPH S. KENDALL, Primary Examiner

U.S. Cl. X.R.

148—6.17